# EUROPEAN PATENT SPECIFICATION

(11) **EP 1 006 821 B1**
(45) Date of publication and mention of the grant of the patent: **17.09.2003**
(21) Application number: 98914523.0
(22) Date of filing: 06.04.1998
(51) Int. Cl.: A41D 7/00, A41H 42/00, A41B 13/08, A41B 9/06

(54) **A CAMISOLE GARMENT**
KAMISOL
VETEMENT CAMISOLE

(30) Priority: 08.04.1997 US 841989; 08.04.1997 US 841958
(43) Date of publication of application: 14.06.2000
(73) Proprietor: Kimberly Clark Worldwide, Inc., Neenah, WI 54956 (US)
(72) Inventor: ALBERTS, Joseph, Richard, Menasha, WI 54952 (US); DREZDZON, Edward, Anthony, II, Appleton, WI 54914 (US); FRIES, Donald, Merlin, Combined Locks, WI 54113 (US); KONETZKE, Richard, Mark, Menasha, WI 54952 (US); KVITEK, Thomas, Theodore, Menasha, WI 54952 (US); MUHLEBACH, Michael, Joseph, Menasha, WI 54952 (US); NELSON, Michael, Joseph, Neenah, WI 54956 (US); RABE, Gerald, Leigh, Appleton, WI 54915 (US); RIBBLE, Brendon, Frank, Menasha, WI 54952 (US); ROTH, James, Frederick, Appleton, WI 54915 (US); WITTMANN, Jon, Mark, Combined Locks, WI 54113 (US); ROSCH, Paulette, Mary, Sherwood, WI 54169 (US); MCPHILLIAMY, Ingrid, Christine, Chicago, IL 60613 (US); ROBINSON, Mark, Louis, Appleton, WI 54914 (US)
(74) Representative: Davies, Christopher Robert
(86) International application number: US9806785
(87) International publication number: WO98044816

(56) References cited:
- DE-A- 1 925 303
- GB-A- 486 475
- US-A- 2 760 202

## Description

### Background of the Invention

This invention pertains to elasticized camisole garments particularly, though not exclusively, intended for the use of bathers or swimmers and relates to the kind which are typically disposable and primarily for children.

Currently, disposable waste containment articles find widespread use in the areas of adult care, infant care, and child care, and have generally replaced reusable cloth articles. Disposable diapers, for example, have met a particular need and have become very popular. Disposable training pants have also met a particular need and have become popular. However, once a child desires to travel to a swimming pool or beach, the child requires a waste containment garment for possible "accidents" during such travel as well as during the child's or adults activities at the pool or beach. As part of a disposable swim wear, a disposable girl's top is desired by the child, the parent of that child, or both.

In fitting the child, one form of the top is a fully elasticized structure which extends from just about the top of the arm pit to just above the wearer's stomach or down to the waist, as described in UK Patent No. GB-486475.
One problem in the fit of the elastidzed material occurs when it has consisted of a bulked web composite such as described in U.S. Patent No. 4,606,964. The bottom edge of the top has a tendency to curl up and fold over. This creates a poor appearance, and the camisole garment tends to ride up on the wearer.

This invention pertains to a continuous process for the manufacture of garments such as sleeveless tops, shirts; and blouses intended for everyday wear, and more particularly to a process for the manufacture of camisole-type garments.

Manufacturers are always looking for new, cost-effective, high-speed continuous processes for manufacturing inexpensive clothing, both disposable and reusable garments, for everyday use. In addition, consumers are interested in active wear that is comfortable and relatively inexpensive, especially if the garments are for children.

Previous methods used in clothing manufacture require pieces of fabric or similar such material to be cut into specific patterns. The pieces are then sewn together in a multistep process for assembly into articles of clothing. Such processes are labor intensive. The process speeds typically depend on the speed of the final sewing stages.

### Summary of the Invention

Thus, there is a need to provide an improved child's swimming apparel that minimizes the bottom rollover tendency during wearing while maintaining proper coverage. In addition, the top needs to be easy to place on the wearer, durable during wear, and, because the top is disposable, low in cost In response to these needs, an improved elasticized top has been discovered.

Thus, there is a need to provide a comfortable and inexpensive active wear clothing, specifically tops that minimize the bottom rollover tendency during wearing while maintaining proper coverage. In addition, the top needs to be easy to place on the wearer and durable during wear. In response to these needs, an improved cost-effective, high speed process for manufacturing a sleeveless garment, such as a top, shirt, or blouse, has been discovered.

The present invention is for a camisole garment as claimed in claim 1.

One embodiment of the present invention is a continuous process for the manufacture of a camisole garment to be worn about the upper body comprising: providing at least a single layer web of fabric including an upper edge, a lower edge, and a body covering assembly; intermittently cutting the fabric, defining at least one opening in the fabric wherein each opening includes a top edge adjacent to the upper edge of the fabric; folding at least a portion of the fabric between at least one of the openings and the upper edge of the fabric back onto the body covering assembly of the fabric wherein at least one shoulder strap is formed; fastening the folded portion of the fabric to the body covering assembly of the fabric to form a neckline fold; cutting the fabric, defining discrete garment-sized pieces wherein each piece of fabric includes at least one opening, at least one shoulder strap, and two opposing end portions; and folding the discrete garment-sized piece of fabric whereby the two opposing end portions are brought into contact with each other.

Numerous features and advantages of the present invention will appear from the following description. In the description, reference is made to the accompanying drawings which illustrate desired embodiments of the invention. Such embodiments do not represent the full scope of the invention. Reference should therefore be made to the claims herein for interpreting the full scope of the invention.

### Brief Description of the Drawings

The above-mentioned and other features of the present invention and the manner of attaining them will become more apparent, and the invention itself will be better understood by reference to the following description of the invention, taken in conjunction with the accompanying drawings, wherein:
**Fig. 1** is a front view of a top typifying an embodiment of the present invention for a camisole garment.
**Fig. 2** is a front view of a top typifying another embodiment of the present invention for a camisole garment having one shoulder strap.
**Fig. 3** is a back view of a top typifying an embodiment of the present invention showing a refastenable body seam.

### Definitions

Within the context of this specification, each term or phrase below will include the following meaning or meanings:
(a) "**Bonded**" refers to the joining, adhering, connecting, attaching, or the like, of two elements. Two elements will be considered to be bonded together when they are bonded directly to one another or indirectly to one another, such as when each is directly bonded to intermediate elements.
(b) "**Bonded Carded Fabric or Web**" refers to fabric or webs made from staple fibers which are sent through a combing or carding unit, which breaks apart and aligns the staple fibers in the machine direction to form a generally machine direction-oriented fibrous nonwoven web. Such fibers are usually purchased in bales which are place in a picker which separates the fibers prior to the carding unit. Once the web or fabric is formed, it is then bonded by one or more of several known bonding methods. Once such bonding method is powder bonding, wherein a powdered adhesive is distributed through the web or fabric and then activated, usually by heating the fabric and adhesive with hot air. Another suitable bonding method is pattern bonding, wherein heated calender rolls or ultrasonic bonding equipment are used to bond the fibers together, usually in a localized bond pattern, though the fabric can be bonded across its entire surface if so desired. Another suitable and well-known bonding method, particularly when using bi-component staple fibers, is through-air bonding.
(c) "**Camisole**" refers to a sleeveless top garment, similar to a sleeveless undergarment, but which can be worn as an outer garment.
(d) "**Cross Machine Direction**" means the width of the fabric in a direction generally perpendicular to the machine direction.
(e) "**Disposable**" includes being disposed of after use, and not intended to be washed and reused.
(f) "**Disposed**", "**disposed on**", "**disposed with**", "**disposed at**", "**disposed near**", and variations thereof are intended to mean that one element can be integral or unitary with another element, or that one element can be a separate structure joined to or connected to or placed with or placed near another element.
(g) "**Elasticity**" and "**elastic**" include that property of a material by virtue of which it tends to substantially recover to its original size and shape after removal of a force causing deformation of the material.
(h) "**Elastically connected**" and "**elastically connecting**" refer to two elements being separated by and bonded to an elastic member, where the relative position of the two elements may change due to extension of the elastic member.
(i) "**Elongation**" indudes the ratio of the extension of a material to the length of a material prior to the extension. Elongation is expressed in percent.
(j) "**Extension**", "**extend**", and "**extended**" include the change in length of a material due to stretching. Extension is expressed in units of length.
(k) "**Fabric**" is used to refer to all of the woven, knitted. and nonwoven webs.
(I) "**Flexible**" refers to materials or fabrics that are compliant and readily conform to the general shape and contours of an individual's body.
(m) "**Force**" indudes a physical influence exerted by one body on another which produces acceleration of bodies that are free to move and deformation of bodies that are not free to move. Force is expressed in Newtons (grams-force).
(n) "**Foreshortened**" and "**foreshortening**" include to shorten beforehand, that is, before a subsequent step.
(o) "**Front**" and "**back**" are used to designate relationships relative to the garment itself, rather than to suggest any position the garment assumes when it is positioned on a wearer.
(p) "**Gatherable**" material is one which, when bonded to the reticular web with the latter under tension, will gather, with the formation of puckers or gathers, to accommodate contraction of the reticulated web upon release of the tensioning forces.
(q) "**Machine Direction**" means the length of a fabric in the direction in which it is produced or the length of fabric moving in the direction of the machine operations.
(r) "**Meltblown Fibers**" means fibers formed by extruding a molten thermoplastic material through a plurality of fine, usually circular, die capillaries as molten threads or filaments into converging high velocity, usually hot gas (e.g. air) streams which attenuate the filaments of molten thermoplastic material to reduce their diameter, which may be to microfiber diameter. Thereafter, the meltblown fibers are carried by the high velocity gas stream and are deposited on a collecting surface to form a web of randomly disbursed meltblown fibers. Such a process is disclosed, for example in U.S. Patent 3,849,241 to Butin et al. Meltblown fibers are microfibers which may be continuous or discontinuous, are generally smaller than 10 microns in average diameter, and are generally tacky when deposited onto a collecting surface.
(s) "**Member**" when used in the singular can have the dual meaning of a single element or a plurality of elements.
(t) "**Multi-layer Laminate**" means a laminate wherein some of the layers are spunbond and some are meltbtown such as a spunbond/meltblown/spunbond (SMS) laminate and other as disclosed in U.S. Patent 4,041,203 to Brock et al., U.S. Patent 5,169,706 to Collier et al., U.S. Patent 5,145,727 to Potts et al., U.S. Patent 5,178,931 to Perkins, et al., and U.S. Patent 5,188,885 to Timmons et al. Such a laminate may be made by sequentially depositing onto a moving forming belt first a spunbond fabric layer, then a meltblown fabric layer and last another spunbond layer and then bonding the laminate in a manner described below. Alternatively. the fabric layers may be made individually, collected in rolls, and combined in a separate bonding step. Such fabrics usually have a basis weight of from about 4 to 400 gsm (about 0.1 to 12 osy), or more particularly from about 25 to 100 gsm (about 0.75 to about 3 osy). Multi-layer laminates may also have various numbers of meltblown layers or multiple spunbond layers in many different configurations and may include other materials like films or coform materials.
(u) **"Neckable Material"** means any material which can be necked.
(v) **"Necked Material"** refers to any material which has been vonstricted in at least one dimension by processes such as, for example, drawing or gathering.
(w) "**Non-elastic**" or "**Inelastic**" refers to any material that does not fall within the definition of "elastic".
(x) "**Nonwoven fabric or web**" means a web having a structure of individual fibers or threads which are interlaid, but not in an identifiable manner as in a knitted fabric. Nonwoven fabrics or webs have been formed from many processes such as, for example, meltblowing processes, spunbonding processes, and bonded carded web processes. The basis weight of nonwoven fabrics is usually expressed in ounces of material per square yard (osy) or grams per square meter (gsm) and the fiber diameters are usually expressed in microns.
(y) "**Operatively joined**" with reference to the attachment of an elastic member to another element means that the elastic member when attached to or connected to or treated with heat with the element gives that element elastic properties. With reference to the attachment of a non-elastic member to another element, it means that the member and element can be attached in any suitable manner that permits or allows them to perform the intended or described function of the joinder. The joining, attaching, connecting or the like can be either directly, such as joining either member directly to an element, or can be indirectly by means of another member or element disposed between the first member and the first element.
(z) "**Pattern**" includes any geometric or non-geometric form that can include, among others, a series of connected or unconnected lines or curves, a series of parallel or nonparallel or intersecting lines or curves, a series of linear or curvilinear lines, and the like, or any combinations thereof. The pattern can include a repeating form and/or non-repeating form.
(aa) "**Ruffles**" includes the region of the material which lies outside the outermost elastic and includes no elastic material. That is, no elastic material is present or the elastic material which was present has been rendered inelastic.
(bb) "**Rupture**" includes the breaking or tearing apart of a material. In tensile testing, rupture refers to the total separation of a material into two parts, either all at once or in stages, or the development of a hole in some materials.
(cc) "**Stretch bonded**" refers to an elastomeric strand being bonded to another member while the elastomeric strand is elongated at least 25 percent of its relaxed length. Desirably, the term "stretch bonded" refers to the situation wherein the elastomeric strand is elongated at least 50 percent, more desirably at least 300 percent, of its relaxed length when it is bonded to the other member.
(dd) "**Stretch bonded laminate**" ("**SBL**") refers to a composite material having at least two layers in which one layer is a gatherable layer and the other layer is a stretchable, that is, elastic, layer. The layers are joined together when the stretchable layer is in a stretched condition so that upon relaxing the layers, the gatherable layer is gathered.
(ee) "**Spunbonded fibers**" refers to small diameter fibers which are formed by extruding molten thermoplastic material as filaments from a plurality of fine, usually circular capillaries or spinneret with the diameter of the extruded filaments then being rapidly reduced as by, for example, as disclosed in in U.S. Patent 4,340,563 to Appel et al., and U.S. Patent 3,692,618 to Dorschner et al., U.S. Patent 3, 802,817 to Matsuki et al., U.S. Patents 3,338,992 and 3,341,394 to Kinney, U.S. Patent 3,502,763 to Hartman, and U.S. Patent 3,542,615 to Dobo et al. Spunbond fibers are generally not tacky when they are deposited onto a collecting surface. Spunbond fibers are generally continuous and have average diameters (from a sample of at least 10) larger than 7 microns, more particularly, between about 10 and 20 microns.
(ff) "**Tension**" includes a uni-axial force tending to cause the extension of a body or the balancing force within that body resisting the extension.
(gg) "**Two-dimensional**" refers to a garment, such as a diaper, that can be opened and laid in a flat condition without destructively tearing any structure. This type of garment does not have continuous leg and waist openings when opened and laid flat, and requires a fastening device, such as adhesive tapes, to attach the garment about the wearer.
(hh) "**Three-dimensional**" refers to a finished garment similar to shorts or pants in that they have continuous leg and waist openings that are bounded by the material of which the garment is made. This type of garment can be opened and laid flat only by destructively tearing it This type of garment may or may not have manually tearable seams.
(ii) "**Ultimate elongation**" includes the elongation at the point of rupture.

These definitions are not intended to be limiting and these terms may be defined with additional language in the remaining portion of the specification.

Referring to **Fig. 1**, one embodiment of the present invention is a camisole garment **2** for wearing about the body comprising an elastic top **10** having a body covering assembly **11,** an upper body opening **12** and a lower body opening **14,** each opening **12** and **14** having an edge **4** or **6,** respectively, about its perimeter. The top **10** comprises an outer cover **16** and bodyside liner **18** both of which generally cover a series of body elastics **20.**

The body elastics **20** circumferentially surround the body of the wearer to form a relatively elastic region **22** of the top **10.** The body elastics **20** act independently to conform to the contours of various body types and builds. This provides a smooth, conformable, and comfortable fit within a given chest size range.

About the lower body opening **14**, below and adjacent the relatively elastic region **22,** there is formed at the lower edge **6** a relatively inelastic lower edge region **30.** In addition, about the upper body opening **12,** above and adjacent the relatively elastic region **22,** there is formed at the upper edge **4** a relatively inelastic upper edge region **24.** The relatively inelastic upper edge region **24** and the relatively inelastic lower edge region **30** form areas of ruffles on the top **10.** The relatively inelastic upper edge region **24** and the relatively inelastic lower edge region **30** each have a width ranging from 0.64 cm to 10.2 cm (0.25 to 4.0 inches). The widths of these regions **24** and **30** are independent of each other. The desired width of the relatively inelastic upper edge region **24** and the relatively inelastic lower edge region **30** is between 0.64 cm to 5.1 cm (0.25 to 2.0 inches), and more desirably, from 0.64 cm to 2.5 cm (0.25 to 1.0 inch).

A pair of openings **32** and **34,** serving as arm holes **33** and **35,** respectively, are cut out of the relatively elastic region **22,** desirably adjacent or near the inelastic upper region **24.** The top edges **36** and **38** of the openings **32** and **34,** respectively, may be located from 0.64 cm to 5.1 cm (0.25 inch to 2.0) inches below the relatively inelastic upper edge region **24.** The openings **32** and **34** are desirably located in opposing positions. The openings **32** and **34** may be slits, circular holes, square holes, oval holes, irregular shaped holes, or the like.

In a top **10** intended for a 25 pound girl, the body elastics **20** are about 406 mm (16 inches) long unstretched. For a top **10** does not cover the girl's stomach, the height of the top **10** is about 146 mm (5.75 inches) wide. For a top **10** that does cover to the waist the height may be about 229 mm (9.50 inches) wide.. If it does extend to the waist, the top **10** may be fastened to a bottom or pant-type garment.

The top **10** includes a pair of straps **26** and **28** which help hold the camisole garment **2** in place. The straps **26** and **28** are formed by the fabric **3** located above the top edges **36** and **38** of the arm holes **32** and **34** and the upper edge **4**. The straps **26** and **28** may be formed by folding the upper edge **4**, the relatively inelastic upper edge region **24**, and a portion of the relatively elastic region **22** back onto relatively elastic region **22** of the top **10.** Desirably, the outer cover **16** is folded back onto itself, exposing a portion of the bodyside liner **18** and creating a neckline edge fold **40.** In an alternative embodiment, the bodyside liner **18** is folded back onto itself, positioning a portion of the outer cover **16** against the body of the wearer.

In an alternative embodiment of the present invention (See **Fig. 2**), the body covering assembly **11** includes only one opening **32** in the relatively elastic region **22** of the body covering assembly **11,** and adjacent to the relatively inelastic upper edge region **24** of the fabric **3.** Desirably, the outer cover **16** is folded back onto itself, exposing a portion of the bodyside liner **18** and creating a neckline edge fold **40.** In an alternative embodiment, the bodyside liner **18** is folded back onto itself, positioning a portion of the outer cover **16** against the body of the wearer. Only one shoulder strap **26** is formed on the camisole garment **2.**

In a desired embodiment, the folded material **5** which includes the upper edge **4** and the portion of the body covering assembly **11** lies on the outer surface **37** of the finished garment **2**. In another embodiment, the folded material **5** lies on the inner surface **39** of the finished garment **2**.

The neckline edge fold **40** is maintained by bonding the folded portion to the top **10** thereby forming a non-refastenable seam. The non-refastenable seam may be formed by any suitable means such as ultrasonic seating, adhesive bonding, heat sealing, or the like. One suitable method of forming such seams is disdosed in U.S. Patent 4,938,753.

Both the outer cover **16** and the bodyside liner **18** are desirably compliant and soft feeling to the wearer. The following description of materials from which the outer cover 16 may be formed may also be used to form the material of the bodyside liner **18**.

The outer cover **16** may be any suitable gatherable material, such as a woven material, a nonwoven material, a fibrous or a polymeric film material and may be, although they need not necessarily be, an elastic material. Suitable fibrous gatherable webs may utilize any suitable natural and/or synthetic fibers, for example, woven or nonwoven webs of fibers made of acrylic polymers, polyester, polyamide, glass, polyolefins. e.g., polyethylene and polypropylene, cellulosic derivatives such as rayon, cotton, silk, wool, pulp, paper and the like, as well as blends or combinations of any two or more of the foregoing. The gatherable webs may also comprise polymeric film layers such as polyethylene, polypropylene, polyamide, polyester, acrylic polymers, and compatible mixtures, blends and copolymers thereof.

The outer cover **16** may be liquid pervious, permitting liquids to readily penetrate into its thickness, or impervious, resistant to the penetration of liquids into its thickness. Outer cover **16** may be made from a wide range of materials, such as natural fibers (e.g. wood or cotton fibers), synthetic fibers (e.g. polyester or polypropylene fibers) or from a combination of natural and synthetic fibers or reticulated foams and apertured plastic films. The outer cover **16** may be woven, nonwoven or film such as spunbonded, carded, or the like. A suitable outer cover **16** is carded, and thermally bonded by means well known to those skilled in the fabric art Alternatively, the outer cover **16** is derived from a spunbonded web. In a desired embodiment, the outer cover **16** is spunbonded polypropylene nonwoven, meltblown polypropylene nonwoven and spunbonded polypropylene nonwoven laminate (SMS). The basis weight per ply of SMS is 14 to 34 gsm (0.4 to 1.0 osy) more desirably to about 20 gsm (0.6 osy) and is made with about 86% spunbonded nonwoven and 14% meltblown nonwoven. A pigment such as titanium dioxide may be incorporated into the outer cover **16** and bodyside liner **18**. A variety of pigment colorants may also be added. Such spunbonded meltblown nonwoven laminate material is available from Kimberly-Clark Corporation, Roswell, GA. The basis weight of the SMS material may vary from 1.4 to 34 gsm (0.4 to 1.0 osy).

In other desired embodiments, the outer cover **16** is spunbonded polypropylene nonwoven with a wireweave bond pattern having a grab tensile of 8.6 kg (19 pounds) as measured by ASTM D1682 and D1776, a Taber 40 cyde abrasion rating of 3.0 as measured by ASTM D1175 and Handle-O-Meter MD value of 6.6 grams and CD value of 4.4 grams using TAPPI method T402. Such spunbonded material is available from Kimberly-Clark Corporation. Roswell, GA. The outer cover **16** has a weight of from 17 gsm (0.5 osy) to 50 gsm (1.5 osy), desirably about 24 gsm (0.7 osy).

The outer cover **16** may be constructed of a single spunbonded polypropylene nonwoven web having a basis weight of 17 gsm (0.5 osy) to 51 gsm (1.5 osy) in the structure of the top **10**, the outer cover **16** desirably comprises a material having a basis weight of from 17 gsm (0.5 osy) to 51 gsm (1.5 osy). Lesser basis weights may be used in the other regions of the article. Since the camisole garment **2** is typically intended for active wear, the outer cover **16** or portions thereof, can be made of materials having a basis weight and bonded structure which resist abrasion.

The bodyside liner **18** may be any soft, flexible, porous sheet. Again, the bodyside liner **18** must permit submersion in fresh water or salt water or treated water (chlorinated or bromated) and still retain its integrity.

The bodyside liner **18** may comprise, for example, a nonwoven web or sheet of a spunbonded, meltblown or bonded-carded web composed of synthetic polymer filaments, such as polypropylene, polyethylene, polyesters or the like, or a web of natural polymer filaments such as rayon or cotton. The bodyside liner 18 may be selectively embossed or perforated with discrete slits or holes extending therethrough.

A suitable adhesive for adhering the laminate layers is H2096 hot melt adhesive that can be obtained from Findley Adhesives, Inc. of Wauwatosa, Wisconsin.

The outer cover **16** and bodyside liner **18** may be further dyed, pigmented, or imprinted with any suitable color or pattern. Desirably, the bodyside liner **18** is either dyed, pigment, or printed with a material which does not irritate or bleed the color onto the skin of the wearer.

Materials suitable for use as the body elastics **20** indude a wide variety, but not limited to, elastic threads, meltblown elastomeric polymer, yam rubber, flat rubber (e.g. as bands), elastic tape, fdm-type rubber, polyurethane, and tape-like elastomer. or foam polyurethane or formed elastic scrim. Each body elastic **20** may be unitary, multi-part, or composite in construction. Threads or ribbons, where used, may be multiple and may be applied as a composite. The elastomerics used in the body elastics **20** may be latent and non-latent.

Desirably, the body elastics **20** are elongated to between 50% to 300%. The elongations may vary for separate elements and still be within the overall elongation for the composite of the elements comprising the body elastics **20.**

The body elastics **20** circumferentially surround the body of the wearer to form a relatively elastic region **22** of the top **10.** The body elastics **20** act independently to conform to the contours of various body types and builds. This provides a smooth, snug, and comfortable fit within a given chest size range.

About the lower body opening **14,** below and adjacent the relatively elastic region **22,** there is formed at the lower edge **6** a relatively inelastic lower edge region **30.** In addition, about the upper body opening **12,** above and adjacent the relatively elastic region **22,** there is formed at the upper edge **4** a relatively inelastic upper edge region **24.** The relatively inelastic upper edge region **24** and the relatively inelastic lower edge region **30** form areas of ruffles on the top **10.** The relatively inelastic upper edge region **24** and relatively inelastic lower edge region **30** each have a width ranging from 0.64 cm to 10.2 cm (0.25 to 4.0 inches). The widths of these regions **24** and **30** are independent of each other. The desired width of the relatively inelastic upper edge region **24** and the relatively lower edge region **30** is between 0.64 to 10.2 cm (0.25 to 2.0 inches), and more desirably, from 0.64 to 2.5 cm (0.25 to 1.0 inch).

As illustrated most dearly in **Fig. 1**, opposing end portions **48** and **50** of top **10** may be bonded together in the finished top **10** to form a body seam **42** that is non-refastenable. The non-refastenable body seam **42** may be formed by any suitable means such as ultrasonic sealing, adhesive bonding, heat sealing, or the like, as discussed above. In other embodiments, the opposing end portions **48** and **50** of the top **10** may be held together in the finished top **10** to form a refastenable body seam **42.**

Refastenable means for securing the opposing end portions **48** and **50** of the top **10** include adhesives and mechanical type fasteners **96.** Mechanical type fasteners include buttons, button holes, snaps, buckles, clasps, hooks and loops, end extensions, tabs, and the like which are designed or adapted to interlock or engage some type of a complimentary device or the outer cover **16** of the top **10.** In addition, elasticized fasteners may also be used in assuring better fit of the camisole garment **2.**

The structure material of the top **10** desirably has stretch characteristics in a first direction such that it is capable of from 10 to 500 percent elongation and upon release of tension will recover at least 55 percent of its elongation. It is generally desired that the structure material of the top **10** in the first direction be capable of between 50 and 300 percent elongation, particularly at least 125 percent elongation and recovery upon release of tension of at least 80 percent of its elongation.

As described previously, the top **10** may be formed of a material capable of stretching in one direction or capable of stretching in two perpendicular directions. One suitable one-directional stretch material is disclosed in U.S. Patent 4,720,415.

The one-directional stretch material may comprise a composite material including at least one gatherable web bonded to at least one elongated elastic web. The elastic web may be an elastic film or nonwoven fibrous elastic webs such as meltblown elastomeric fibrous webs. In one embodiment, the top **10** comprises a stretch bonded laminate formed of a pre-stretched elastic meltblown inner layer sandwiched between and attached to a pair of spunbond polypropylene nonwoven webs, each web having a basis weight of about 14 gsm (0.4 osy). Suitable elastic materials can be purchased from the Shell Chemical Company of Houston, Texas under the trade name Kraton. Other suitable one-directional stretch materials are disclosed in U.S. Patents 4,606,964 issued August 19, 1986, to Wideman and 4,657,802 issued April 14, 1987, to Monnan.

Suitable two-directional stretch materials for the body elastics 20 are disclosed in U.S. Patents 5,114,781 and 5,116,662.

A two-directional stretch material may comprise a composite material including a neckable material and an elastic sheet, which may be formed by meltblowing or extrusion. Neckable materials are those which may be constricted in at least one dimension by applying a tensioning force in a direction perpendicular to the desired direction of neck-down, and may include a spunbonded, meltblown or bonded carded web. The tensioned, necked neckable material may be joined to the elongated elastic sheet at spaced locations arranged in a nonlinear configuration.

Another two-directional stretch composite material may comprise one or more layers of reversibly necked material joined to one or more layers of elastic sheet at spaced locations. Reversibly necked materials are those that have been treated, such as with heat, while necked to impart memory to the material so that, when a force is applied to extend the material to its pre-necked dimensions, the treated, necked portions will generally recover to their necked dimensions upon termination of the force.

Desirably, the material stretches in horizontal direction only, that is, around the body. If the material is elastic in both directions, it is desirable to limit the stretch in the vertical direction to less than 20% under normal tensions.

Alternately, the body elastics **20** may be formed of a dry-spun coalesced multi-filament elastomeric thread sold under the tradename LYCRA and available from I.E. Du Pont de Nemours and Company. still altemately, the elastics may be formed of other typical elastics utilized in the diaper-making art, such as a thin ribbon of elastic material as disclosed in U.S. Patent 4,940,464.

Elasticity could also be imparted to the structure material of the top **10** by extruding a hot melt elastomeric adhesive between the outer cover **16** and the bodyside liner **18.** Other suitable elastic gathering means are disclosed in U.S. Patents No. 4,938,754 to Mesek and 4,388,075 to Mesek et al.

In forming the top **10** structure material, the body elastics **20** may be individually laid on one of the adjacent gatherable layers (outer cover 16 or bodyside liner **18**) and the other gatherable layer web applied over the elastics to bond the first layer. Alternatively, only one gatherable layer, e.g., the outer cover **16**, may be employed and the body elastics **20** bonded to one side, desirably the bodyside, of the outer cover **16**. In such an embodiment, the body elastics **20** are left exposed on one side of the outer cover **16**.

Another embodiment of the present invention is a camisole garment **2** for wearing about the body comprising a body covering assembly **11** having an upper body opening **12** and a lower body opening **14**. (See **Fig. 3**) The upper body opening **12** has an upper edge **4** about its perimeter. The lower body opening **14** has a lower edge **6** about its perimeter.

The body covering assembly **11** comprises a single layer web of fabric **3** between the upper edge **4** and the lower edge **6** of the fabric **3**; at least two opposing openings **32** and **34** in the body covering assembly **11**; two opposing end portions **48** and **50** between the upper edge **4** and the lower edge **6** of the fabric **3**; and, a neckline edge fold **40** created by folding the upper edge **4** and a portion of the body covering assembly **11** above the opposing openings **32** and **34** over onto the body covering assembly **11**. In the desired embodiment, the folded material **5** which includes the upper edge **4** and the portion of the body covering assembly **11** lies on the outer surface 37 of the finished garment **2**. In another embodiment, the folded material **5** lies on the inner surface **39** of the finished garment **2**.

The single layer web of fabric **3** used in the process may be any suitable material, such as a woven material, a nonwoven material, a fibrous or a polymeric film material and may include an elastic material. Suitable fibrous webs may utilize any suitable natural and/or synthetic fibers, for example, woven or nonwoven webs of fibers made of acrylic polymers, polyester, polyamide, glass, polyolefins, e.g., polyethylene and polypropylene, cellulosic derivatives such as rayon, cotton, silk, wool, pulp, paper and the like, as well as blends or combinations of any two or more of the foregoing. The web may also comprise a polymeric film layer such as polyethylene, polypropylene, polyamide, polyester, acrylic polymers, and compatible mixtures, blends and copolymers thereof.

The fabric **3** may be liquid pervious, permitting liquids to readily penetrate into its thickness, or impervious, resistant to the penetration of liquids into its thickness. The fabric **3** may also be made from a wide range of materials, such as natural fibers (e.g. rayon, wood, or cotton fibers), synthetic fibers (e.g. polyester or polypropylene fibers) or from a combination of natural and synthetic fibers or reticulated foams and apertured plastic films. The fabric 3 may be woven, nonwoven or film such as spunbonded, meltblown, bond-carded, or the like. A suitable fabric **3** is carded, and thermally bonded by means well known to those skilled in the fabric art.

The fabric **3** may be further dyed, pigmented, or imprinted with any suitable color. Desirably, the fabric **3** is either dyed, pigmented, or printed with a material which does not irritate or bleed the color onto the skin of the wearer.

The body seam **42** of the camisole garment **2** may comprise a non-refastenable body seam **42** by engaging the two opposing end portions **48** and **50**. (See **Fig. 1**) The non-refastenable body seam **42** may be formed by any suitable means such as ultrasonic sealing, adhesive bonding, heat sealing, or the like, as discussed above. In other embodiments, the opposing end portions **48** and **50** of the top **10** may be held together in the finished top **10** to form a refastenable body seam **42.** (See **Fig. 3**)

In another embodiment of the present invention, the body seam **42** of the camisole garment **2** comprises a refastenable body seam **42** by refastenably engaging the two opposing end portions **48** and **50**. Refastenable means for securing the opposing end portions **48** and **50** of the top **10** include adhesives and mechanical type fasteners **96**. Mechanical type fasteners include buttons, button holes, snaps, buckles, clasps, hooks and loops, end extensions, tabs, and the like which are designed or adapted to interlock or engage some type of a complimentary device or the outer cover **16** of the top **10**. In addition, elasticized fasteners may also be used in assuring better fit of the camisole garment **2**.

In another embodiment of the present invention, the camisole garment **2** for wearing about the body comprises a body covering assembly **11** having an upper body opening **12** and a lower body opening **14**. (See **Fig. 2**) The upper opening **12** has an upper edge **4** about its perimeter. The lower opening **14** has a lower edge **6** about its perimeter.

The body covering assembly **11** comprises a single layer web of fabric **3** between the upper edge **4** and the lower edge **6**; at least one opening **32** in the body covering assembly **11** adjacent to the upper edge **4** of the fabric **3**; two opposing end portions **48** and **50** (not shown) between the upper edge **4** and the lower edge **6**; and, a neckline edge fold **40** created by folding the upper edge **4** and a portion of the body covering assembly **11** above the opening **32** over onto the body covering assembly **11.**

In the desired embodiment, the folded material **5** which includes the upper edge **4** and the portion of the body covering assembly **11** lies on the outer surface **37** of the finished garment **2.** In another embodiment, the folded material **5** lies on the inner surface **39** of the finished garment **2**.

The camisole garment **2** may further comprise a non-refastenable body seam **42** by non-refastenably engaging the two opposing end portions **48** and **50**. The non-refastenable body seam **42** may be formed by any suitable means such as ultrasonic sealing, adhesive bonding, heat sealing, or the like, as discussed above. In other embodiments, the opposing end portions **48** and **50** of the top **10** may be held together in the finished top **10** to form a refastenable body seam **42**.

In another embodiment of the present invention, the body seam **42** of the camisole garment **2** comprises a refastenable body seam **42** by refastenably engaging the two opposing end portions **48** and **50**. Refastenable means for securing the opposing end portions **48** and **50** of the top **10** include adhesives and mechanical type fasteners **96**. Mechanical type fasteners include buttons, button holes, snaps, buckles, clasps, hooks and loops, end extensions, tabs, and the like which are designed or adapted to interlock or engage some type of a complimentary device or the outer cover **16** of the top **10**. In addition, elasticized fasteners may also be used in assuring better fit of the camisole garment **2**.

The present invention relates to a camisole garment **10** for wearing about the body comprising a body covering assembly **11** having an upper body opening **12** and a lower body opening **14**, wherein each opening having an edge about its perimeter. The body covering assembly **11** comprises: a relatively elastic region **22** between the upper edge **4** and the lower edge **6**; a relatively inelastic lower edge region **30** between the relatively elastic region **22** and the lower edge **6** wherein the lower edge region **30** is relatively inelastic compared to the relatively elastic region **22**, and the lower edge region **30** further being from 0.6 to 10 cm (0.25 to 4.0 inches) in width; a relatively inelastic upper edge region **24** between the relatively elastic region **22** and the upper edge **4** wherein the upper edge region **24** is relatively inelastic compared to the relatively elastic region **22**, and the upper edge region **24** further being 0.6 to 10 cm (0.25 to 4.0 inches) in width; at least two opposing openings **32** and **34** in the relatively elastic region **22**; and, two opposing end portions **48** and **50** of the body covering assembly **11** between the upper edge **4** and the lower edge **6** engaged to form a body seam **42.**

The camisole garment **10** may further comprise a neckline edge fold **40** created by folding over the upper edge **4,** the relatively inelastic upper edge region **24** and a portion of the relatively elastic region **22** above the opposing openings **32** and **34.** The camisole garment **10** may comprise an outer cover **16** and a bodyside liner **18,** both of which cover a series of body elastics **20** which circumferentially surround the body to form the relatively elastic region **22.**

In the present invention, the two opposing end portions **48** and **50** of the garment **10** may be refastenably engaged to form a refastenable body seam **42.** In the alternative, the two opposing end portions **48** and **50** of the garment **10** may be non-refastenably engaged to form a non-refastenable body seam **42.**

The outer cover **16** of the camisole garment **10** may be a gatherable material; a woven material; a nonwoven material; a polymeric film material; a fibrous material; or, an elastic material. The outer cover **16** may be a spunbonded polypropylene nonwoven material, meltblown polypropylene nonwoven material, or spunbonded polypropylene nonwoven material laminate.

The outer cover **16** may be comprised of acrylic polymer, polyester, polyamide, glass, polyethylene, polypropylene, rayon, cotton, silk, wool, pulp, paper, or a blend or combination of two or more of the foregoing. Alternatively, the outer cover 16 may comprise acrylic polymer, polyester, polyamide, polyethylene, polypropylene, or a compatible mixture, blend or copolymer thereof. The outer cover **16** may have a basis weight of from 14 to 34 gsm (0.4 to 1.0 ounces per square yard) and contain about 86% spunbonded polypropylene nonwoven material and about 14% meltblown polypropylene nonwoven material.

The bodyside liner **18** of the camisole garment **10** may be a soft, flexible porous sheet which permits submersion in fresh water, salt water, chlorinated water or brominated water and thereafter retains its integrity. The body liner **18** may comprise a nonwoven or sheet of spunbonded, meltblown or bonded-carded web composed of polypropylene, polyethylene, polyester, rayon, or cotton filaments.

The body elastics **20** are elastic threads, yam rubber, flat rubber, elastic tape, polyurethane, or foamed elastic scrim. The body elastics **20** are elongated to between 50% to 300%.

The body covering assembly **11** of the camisole garment **10** may be made of materials having stretch characteristics such that the body covering assembly is capable of between 50% to 300% elongation, and recovery, upon release of tension, of at least 80% of its elongation. The body covering assembly **11** may be made of materials capable of stretching in one direction or of materials capable of stretching in two substantially perpendicular directions.

Another embodiment of the present invention is a camisole garment **10** for wearing about the body comprising a body covering assembly **11** having an upper body opening **12** and a lower body opening **14,** wherein each opening having an edge about its perimeter. The body covering assembly **11** comprises: a single layer web of fabric **3** between the upper edge **4** and the lower edge **6;** at least two opposing openings **32** and **34** in the body covering assembly **11;** two opposing end portions **48** and **50** between the upper edge **4** and the lower edge **6;** and, a neckline edge fold **40** created by folding the upper edge **4** and a portion of the body covering assembly **11** above the opposing openings **32** and **34.**

The camisole garment **10** further comprises a non-refastenable body seam **42** by engaging the two opposing end portions **48** and **50.** In the alternative, the garment **10** may comprising a refastenable body seam **42** by refastenably engaging the two opposing end portions **48** and **50**.

In still another embodiment, the present invention relates to a camisole garment **10** for wearing about the body comprising a body covering assembly **11** having an upper body opening **12** and a lower body opening **14**, wherein each opening having an edge about its perimeter. The body covering assembly **11** comprises: a single layer web of fabric **3** between the upper edge **4** and the lower edge **6;** at least one opening **32** in the body covering assembly **11** adjacent to the upper edge **4** of the fabric **3;** two opposing end portions **48** and **50** between the upper edge **4** and the lower edge **6;** and, a neckline edge fold **40** created by folding the upper edge **4** and a portion of the body covering assembly **11** above the opening **32.**

The camisole garment **10** may further comprise a non-refastenable body seam **42** by engaging the two opposing end portions **48** and **50**. Alternatively, the camisole garment **10** may further comprise a refastenable body seam **42** by refastenably engaging the two opposing end portions **48** and **50**.

According to another embodiment of the present invention, the camisole garment **10** for wearing about the body comprising a body covering assembly **11** having an upper body opening **12** and a lower body opening **14**, wherein each opening having an edge about its perimeter. The body covering assembly **11** comprises: a relatively elastic region **22** between the upper edge **4** and the lower edge **6**; a relatively inelastic lower edge region **30** between the relatively elastic region **22** and the lower edge **6** wherein the lower edge region **30** is relatively inelastic compared to the relatively elastic region **22,** and the lower edge region **30** further being from 0.6 to 10 cm (0.25 to 4.0 inches) in width; a relatively inelastic upper edge region **24** between the relatively elastic region **22** and the upper edge **4** wherein the upper edge region **24** is relatively inelastic compared to the relatively elastic region **22,** and the upper edge region **24** further being from 0.6 to 10 cm (0.25 to 4.0 inches) in width; at least one opening **32** in the relatively elastic region **22;** and, two opposing end portions **48** and 50 of the body covering assembly **11** between the upper edge **4** and the lower edge **6** engaged to form a body seam **42.**

The camisole garment **10** may further comprise a neckline edge fold **40** created by folding over the upper edge **4,** the relatively inelastic upper edge region **24** and a portion of the relatively elastic region **22** above the opening **32.** The camisole garment **10** may also comprise an outer cover **16** and a bodyside liner **18**, both of which cover a series of body elastics **20** which circumferentially surround the body to form the relatively elastic region **11**.

The two opposing end portions **48** and **50** may be refastenably engaged to form a refastenable body seam **42**. Alternatively, the two opposing end portions **48** and **50** are non-refastenably engaged to form a non-refastenable body seam **42**.

Although the camisole garment **2** of this invention is generally intended to be disposable, any camisole garment which is reusable may take advantage of this invention. Thus, both reusable and disposable items (the latter term meaning items intended to be discarded after a single use rather than being laundered and reused) are provided by the present invention.

The present invention is a continuous process for the manufacture of a camisole garment **2** as shown in **Fig. 1, 2 and 3**. The fabric **3**, or material, used in the process may be a single layer web or a multi-layer laminate web. The fabric **3** is desirably a soft, flexible sheet.

One embodiment of the present invention is a continuous process for the manufacture of a camisole garment **2** (see **Fig. 3**) for wearing about the body comprising a top **10** having a body covering assembly **11**, an upper body opening **12** and a lower body opening **14**, each opening **12** and **14** having an edge **4** or **6**, respectively, about its perimeter. The illustrated top **10** comprises a single layer web of fabric **3**.

The single layer web of fabric **3** used in the process may be any suitable material, such as a woven material, a nonwoven material, a fibrous, or a polymeric film material and may include an elastic material. Suitable fibrous webs may utilize any suitable natural and/or synthetic fibers, for example, woven or nonwoven webs of fibers made of acrylic polymers, polyester, polyamide, glass, polyolefins, e.g., polyethylene and polypropylene, cellulosic derivatives such as rayon, cotton, silk, wool, pulp, paper and the like, as well as blends or combinations of any two or more of the foregoing. The web may also comprise a polymeric film layer such as polyethylene, polypropylene, polyamide, polyester, acrylic polymers, and compatible mixtures, blends and copolymers thereof.

The fabric **3** may be liquid pervious, permitting liquids to readily penetrate into its thickness, or impervious, resistant to the penetration of liquids into its thickness. The fabric **3** may also be made from a wide range of materials, such as natural fibers (e.g. rayon, wood, or cotton fibers), synthetic fibers (e.g. polyester or polypropylene fibers) or from a combination of natural and synthetic fibers or reticulated foams and apertured plastic films. The fabric **3** may be woven, nonwoven or film such as spunbonded, meltblown, bond-carded, or the like. A suitable fabric **3** is carded, and thermally bonded by means well known to those skilled in the fabric art.

The fabric **3** may be further dyed, pigmented, or imprinted with any suitable color. Desirably, the fabric **3** is either dyed, pigmented, or printed with a material which does not irritate or bleed the color onto the skin of the wearer.

A repeating series of pairs of openings **32** and **34** are cut into the fabric **3.** The location of the openings **32** and **34** corresponds to the arm holes **33** and **35,** respectively, in the finished garment **2.** The openings **32** and **34** may be produced by a die cut operation, an ultrasonic operation, or any other suitable method of operation. The openings **32** and **34** can have a variety of shapes ranging from slit, circular, square, oval, irregular, or the like. The pattern is restricted only by fashion and the minimum amount of fabric **3** that must remain having a sufficient integrity to withstand the remaining steps or operations of the process of manufacture. The top edges 36 and 38 of the openings 32 and 34, respectively, may be located from 0.6 to 13 cm (0.25 inch to 5.0 inches) from the upper edge 4.

The portion of the fabric **3** of the body covering assembly **11** between the upper edge **4** and the openings **32** and **34** is folded back onto itself, thereby forming a neckline edge fold **40**. In the desired embodiment, the fabric **3** is folded such that the folded material **5** lies on the outer surface **37** of the finished garment **2**. In another embodiment, the fabric **3** is folded such that the folded material **5** lies on the inner surface **39** of the finished garment **2**.

The folded material **5** is bonded between the openings **32** and **34,** thereby creating shoulder straps **26** and **28.** The shoulder straps **26** and **28** help hold the camisole garment **2** in place. The bonding forms a non-refastenable seam **42.** The non-refastenable seam **42** may be formed by any suitable means such as ultrasonic sealing, adhesive bonding, heat sealing, tape, sewing, or the like accomplished on a continuous or intermittent basis. One suitable method of forming such seams is disclosed in U.S. Patent 4,938,753.

The fabric **3** is then cut into discrete garment-sized pieces wherein each piece contains one pair of openings **32** and **34,** one pair of shoulder straps **26** and **28** and one pair of opposing end portions **48** and **50.** Each piece of fabric **3** is transported, typically by vacuum screens, belts, or conveyors, through folding and redirection operations. Folding and redirection operations are desirably carried out by turn rolls and turn tables, as well as any other known means. The piece of fabric **3** is folded (desirably via a turn roll) so as to bring together the opposing end portions **48** and **50** to form a body seam **42.** The piece of fabric **3** is redirected (or reoriented) to allow easy bonding of the body seam **42.** The piece of fabric **3** is reoriented **90** degrees. The body seam **42** can be a non-refastenable seam or a refastenable seam. Any excess fabric **3** may be removed from the edge **47** of the body seam **42** to reduce and smooth out the body seam **42.** The non-refastenable body seam **42** may be formed by any suitable means such as ultrasonic sealing, adhesive bonding, tape, heat sealing, sewing, or the like.

In other embodiments, the opposing end portions **48** and 50 of the top **10** may be held together in the finished top **10** to form a refastenable body seam **42.** Refastenable means for securing the opposing end portions **48** and **50** of the top **10** include refastenable adhesive systems and mechanical type fasteners **96.** Mechanical type fasteners include buttons, button holes, snaps, buckles, clasps, hooks and loops, end extensions, tabs, and the like which are designed or adapted to interlock or engage some type of a complimentary device or the outer cover **16** of the top **10.** In addition, elasticized fasteners may also be used in assuring better fit of the camisole garment **2.** If the camisole garment **2** includes a refastenable body seam **42,** the refastenable means are desirably strategically placed on the fabric **3** before the fabric **3** is cut into discrete garment-sized pieces. The folding and redirection operations may be eliminated when a refastenable body seam **42** is Included in the camisole garment **2.** There may be packaging reasons for which one would still carry out these two steps.

Another embodiment of the present invention is a continuous process for the manufacture of a camisole garment **2** (see **Fig. 1 and 2**) for wearing about the body comprising an elastic top **10** having a body covering assembly **11**, an upper body opening **12** and a lower body opening **14**, each opening **12** and **14** having an edge 4 or **6**, respectively, about its perimeter. The top **10** comprises an outer cover **16** and bodyside liner **18** both of which generally cover a series of body elastics **20**. The top **10** comprises a multi-layer laminate web of fabric **3.**

Both the outer cover **16** and the bodyside liner **18** are desirably compliant and soft feeling to the wearer. The following description of materials from which the outer cover **16** may be formed may also be used to form the material of the bodyside liner **18**.

A repeating series of pairs of openings **32** and **34** are cut out of the relatively elastic region **22**, of the fabric **3**, desirably near the inelastic upper region **24.** The location of the openings **32** and **34** correspond to the arm holes **33** and **35** in the finished garment **2.** The top edges **36** and **38** of the openings **32** and **34,** respectively, may be located from 0.6 to 5 cm (0.25 inch to 2.0 inches) below the relatively inelastic upper edge region **24.**

The openings **32** and **34,** as discussed above, can have a variety of shapes. The pattern is restricted only by fashion and the minimum amount of fabric **3** that must remain having suffecient integrity to withstand the remaining steps or operations of the process of manufacture. The openings **32** and **34** may be produced by a die cut operation, an ultrasonic operation, or any other suitable method of operation. The. top edges **36** and **38** of the openings **32** and **34,** respectively, may be located from 0.6 to 13 cm (0.25 inch to 5.0 inches) from the upper edge **24.**

The top **10** includes a pair of shoulder straps **26** and **28** which help hold the camisole garment **2** in place. The shoulder straps **26** and **28** are made of the fabric **3** located between the top edges **36** and **38** of the arm holes **32** and **34** and the upper edge 4.
The portion of the fabric **3** is folded such that the folded material **5** lies on the outer surface **37** of the finished garment **2,** wherein the outer cover **16** is folded back onto itself, exposing a portion of the bodyside liner **18** and creating a neckline edge fold **40.** In an alternative embodiment, the portion of the fabric **3** is folded such that the folded material **5** lies on the inner surface **39** of the finished garment **2,** wherein the bodyside liner **18** is folded back onto itself, positioning a portion of the outer cover **16** against the body of the wearer.

The neckline edge fold **40** is maintained by bonding the folded material **5** to the fabric **3** between the openings **32** and **34**, thereby creating the shoulder straps **26** and **28**. The bonding forms a non-refastenable seam **42**. The non-refastenable seam **42** may be formed by any suitable means such as ultrasonic sealing, adhesive bonding, heat sealing, or the like, as discussed above.

The fabric **3** is then cut into discrete garment-sized pieces wherein each piece contains one pair of openings **32** and **34**, one pair of shoulder straps **26** and **28** and one pair of opposing end portions **48** and 50. Each piece of fabric **3** is transported, typically by vacuum screens, belts, or conveyors, through folding and redirection operations. The piece of fabric **3** is folded so as to bring together the opposing end portions **48** and **50** to form a body seam **42**.

The piece of fabric **3** is redirected (or reoriented) to allow easy bonding of the body seam **42**. The body seam **42** can be a non-refastenable seam or a refastenable seam. Any excess fabric **3** may be removed from the edge **47** of the body seam **42** to reduce and smooth out the body seam **42**. The non-refastenable body seam **42** may be formed by any suitable means such as ultrasonic sealing, adhesive bonding, heat sealing, or the like, as discussed above.

In other embodiments, the opposing end portions **48** and **50** of the top **10** may be held together in the finished top **10** to form a refastenable body seam **42**. Refastenable means for securing the opposing end portions **48** and **50** of the top **10** include refastenable adhesive systems and mechanical type fasteners. Mechanical type fasteners include buttons, button holes, snaps, buckles, clasps, hooks and loops, end extensions, tabs, and the like which are designed or adapted to interlock or engage some type of a complimentary device or the outer cover **16** of the top **10**.

In addition, elasticized fasteners may also be used in assuring better fit of the camisole garment **2**. If the camisole garment **2** includes a refastenable body seam **42**, the refastenable means are desirably strategically placed on the fabric **3** before the fabric **3** is cut into discrete garment-sized pieces. The folding and redirection operations are eliminated when a refastenable body seam **42** is included in the camisole garment **2**.

The fabric **3** of the top **10** desirably has stretch characteristics in a first direction such that it is capable of from 10 to 500 percent elongation and upon release of tension will recover at least 55 percent of its elongation. It is generally desired that the structure material of the top **10** in the first direction be capable of between 50 and 300 percent elongation, particularly at least 125 percent elongation and recovery upon release of tension of at least 80 percent of its elongation.

As described previously the top **10** may be formed of a material capable of stretching in one direction or capable of stretching in at least two substantially perpendicular directions. One suitable one-directional stretch material is disclosed in U.S. Patent 4,720,415.

The one-directional stretch material may comprise a composite material including at least one gatherable web bonded to at least one elongated elastic web. The elastic web may be an elastic film or nonwoven fibrous elastic webs such as meltblown elastomeric fibrous webs. In one embodiment, the top **10** comprises a stretch bonded laminate formed of a pre-stretched elastic meltblown inner layer sandwiched between and attached to a pair of spunbond polypropylene nonwoven webs each having a basis weight of about 14 gsm (0.4 osy). Suitable elastic materials can be purchased from the Shell Chemical Company of Houston, Texas under the trade name Kraton. Other suitable one-directional stretch materials are disclosed in U.S. Patents 4,606,964 issued August 19, 1986, to Wideman and 4,657,802 issued April 14, 1987, to Morman.

Suitable two-directional stretch materials for the body elastics **20** are disclosed in U.S. Patents 5,114,781 and 5,116,662.

A two-directional stretch material may comprise a composite material including a neckable material and an elastic sheet, which may be formed by meltblowing or extrusion. Nedcable materials are those which may be constricted in at least one dimension by applying a tensioning force in a direction perpendicular to the desired direction of neck-down, and may include a spunbonded. meltblown or bonded carded web. The tensioned, necked neckable material may be joined to the elongated elastic sheet at spaced locations arranged in a nonlinear configuration.

Another two-directional stretch composite material may comprise one or more layers of reversibly necked material joined to one or more layers of elastic sheet at spaced locations. Reversibly necked materials are those that have been treated, such as with heat. white necked to impart memory to the material so that, when a force is applied to extend the material to its pre-necked dimensions, the treated, necked portions will generally recover to their necked dimensions upon termination of the force.

Desirably, the material stretches in horizontal direction only, that is, around the body. If the material is elastic in both directions, it is desirable to limit the stretch in the vertical direction to less than 20% under normal tensions.

Alternately, the body elastics **20** may be formed of a dry-spun coalesced multi-filament elastomeric thread sold under the tradename LYCRA and available from I.E Du Pont de Nemours and Company. Still alternately, the elastics may be formed of other typical elastics utilized in the diaper-making art, such as a thin ribbon of elastic material as disclosed in U.S. Patent 4,940.464.

Elasticity could also be imparted to the structure material of the top **10** by extruding a hot melt elastomeric adhesive between the outer cover **16** and the bodyside liner **18**. Other suitable elastic gathering means are disclosed in U.S. Patents No. 4,938,754 to Mesek and 4,388,075 to Mesek et at.

In forming the top **10** structure material, the body elastics **20** may be individually laid on one of the adjacent gatherable layers (outer cover **16** or bodyside liner **18**) and the other gatherable layer web applied over the elastics to bond the first layer. Alternatively, only one gatherable layer, e.g., the outer cover **16**, may be employed and the body elastics **20** bonded to one side, desirably the bodyside, of the outer cover **16**. In such an embodiment, the body elastics **20** are left exposed on one side of the outer cover **16**.

One embodiment of the present invention relates to a continuous process for the manufacture of a camisole garment **10** comprising:
a. providing a single layer web of fabric **3** including an upper edge **4**, a lower edge **6**, and a body covering assembly **11**;
b. intermittently cutting the fabric **3**, defining openings **32** and **34** in the fabric 3 wherein each opening **32** and **34** includes a top edge **33** and **35** adjacent to the upper edge **4** of the fabric **3**;
c. folding at least a portion of the fabric **3** between at least one of the openings **32** and **34** and the upper edge **4** of the fabric **3** back onto the body covering assembly **11** of the fabric **3** wherein at least one shoulder strap **26** is formed;
d. fastening the folded portion of the fabric **3** to the body covering assembly **11** of the fabric **3** to form a neckline fold **40**;
e. cutting the fabric **3**, defining discrete garment-sized pieces wherein each piece of fabric **3** includes at least one opening **32**, at least one shoulder strap **26**, and two opposing end portions **48** and **50**;
f. folding the discrete garment-sized piece of fabric **3** whereby the two opposing end portions **48** and **50** are brought into contact with each other;
g. turning the folded discrete garment-sized piece of fabric **3** to move sideways; and,
h. fastening the two opposing end portions **48** and **50** together to form a body seam **42**.

The continuous process may further comprise cutting off excess fabric **47** remaining of the two opposing end portions **48** and **50** adjacent to the body seam **42**. At least one pair of openings **32** and **34** are cut into the fabric **3**. The body seam **42** can be refastenable or non-refastenable.

Another embodiment of the present invention relates to a continuous process for the manufacture of a camisole garment **10** comprising:
a. providing a multi-layer laminate web of fabric **3** including an upper edge **4**, a lower edge **6**, and a body covering assembly **11**;
b. intermittently cutting the fabric **3**, defining openings **32** and **34** in the fabric **3** wherein each opening **32** and **34** includes a top edge **33** and **35** adjacent to the upper edge **4** of the fabric **3**;
c. folding at least a portion of the fabric **3** between at least one of the openings **32** and the upper edge **4** of the fabric **3** back onto the body covering assembly **11** of the fabric **3** wherein at least one shoulder strap **26** is formed;
d. fastening the folded portion of the fabric **3** to the body covering assembly **11** of the fabric **3**;
e. cutting the fabric **3**, defining discrete garment-sized pieces of fabric **3** wherein each piece of fabric **3** includes at least one opening **32**, at least one shoulder strap **26**, and two opposing end portions **48** and **50**;
f. folding the discrete garment-sized piece of fabric **3** whereby the two opposing end portions **48** and **50** are brought into contact with each other;
g. turning the folded discrete garment-sized piece of fabric **3** to move sideways; and,
h. fastening the two opposing end portions **48** and **50** together to form a body seam **42**.

The continuous process may further comprise cutting off the excess fabric **47** remaining on the two opposing end portions **48** and **50** adjacent to the body seam **42.** The body covering assembly **11** comprises a relatively elastic region **22** between a relatively inelastic lower edge region **30** adjacent to the lower edge **6** of the fabric **3** and a relatively inelastic upper edge region **24** adjacent to the upper edge **4** of the fabric **3**. The relatively elastic region **22** comprises body elastics **20** between an outer cover **16** and a bodyside liner **18** and in which the body elastics **20** circumferentially surround a body of a wearer.

The present invention also relates to a continuous process for the manufacture of a camisole garment **10** comprising:
a. providing a single layer web of fabric **3** including an upper edge **4**, a lower edge **6**, and a body covering assembly **11**;
b. intermittently cutting the fabric **3**, defining openings **32** and **34** in the fabric **3** wherein each opening **32** and **34** includes a top edge **33** and **35** adjacent to the upper edge **4** of the fabric **3**;
c, folding at least a portion of the fabric **3** between at least one of the openings **32** and **34** and the upper edge **4** of the fabric **3** back onto the body covering assembly **11** of the fabric **3** wherein at least one pair of shoulder straps **26** and **28** are formed;
d. fastening the folded portion of the fabric **3** to the body covering assembly **11** of the fabric **3** to form a neckline fold **40**;
e. cutting the fabric **3**, defining discrete garment-sized pieces of fabric **3** wherein each piece of fabric **3** includes at least one pair of openings **32** and **34**, at least one pair of shoulder straps **26** and **28**, and two opposing end portions **48** and **50**; and,
f. folding the discrete garment-sized piece of fabric **3** whereby the two opposing end portions **48** and **50** are brought into contact with each other.

However, the discrete garment-sized piece of fabric **3** does not need to be folded, nor does the two opposing end portions **48** and **50** have to be brought into contact with each other during the process of the present invention. The mechanical fasteners **96**, when used, can be applied during the process of the present invention and the opposing end portions **48** and **50** need never be brought into contact with each other prior to use.

The continuous process may further comprise cutting off excess fabric **47** remaining of the two opposing end portions **48** and **50** adjacent to the body seam **42**. The body seam **42** may be refastenable or non-refastenable. The continuous process may also further comprise turning the folded discrete garment-sized piece of fabric **3** to move sideways.

The present invention relates to a continuous process for the manufacture of a camisole garment **10** comprising:
a. providing a multi-layer laminate web of fabric **3** including an upper edge **4**, a lower edge **6**, and a body covering assembly **11**;
b. intermittently cutting the fabric **3** defining openings **32** and **34** in the fabric **3** wherein each opening **32** and **34** includes a top edge **33** and **35** adjacent to the upper edge **4** of the fabric **3**;
c. folding at least a portion of the fabric **3** between at least one of the openings **32** and **34** and the upper edge **4** of the fabric **3** back onto the body covering assembly **11** of the fabric **3** wherein at least one pair of shoulder straps **26** and **28** are formed:
d. fastening the folded portion of the fabric **3** to the body covering assembly **11** of the fabric **3;**
e. cutting the fabric **3,** defining discrete garment-sized pieces of fabric **3** wherein each piece of fabric **3** includes at least one pair of opposing openings **32** and **34,** at least one pair of shoulder straps **26** and **28,** and two opposing end portions **48** and **50;** and,
f. folding the discrete garment-sized piece of fabric **3** whereby the two opposing end portions **48** and **50** are brought into contact with each other.

The foregoing detailed description has been for the purpose of illustration. Thus, a number of modifications and changes may be made without departing from the spirit and scope of the present invention. For instance, alternative or optional features described as part of one embodiment can be used to yield another embodiment Therefore, the invention should not be limited by the specific embodiments described, but only by the claims.

### Example

The material used to obtain this example consists of a laminate made of 2 facings of 20 gsm (0.6 osy) nonwoven material covering 470 decitex LYCRA elastic strands placed about 3 strands per cm width (7 strands per inch width) of material. The elastic strands are adhesively attached using an add-on of 5 gsm. The elastics are also applied at 150% to 170% stretch. The width of the final laminate is 10cm (4 inches) excluding any non-elasticized ruffle that is added.

The ruffle is formed on the edge of the material by eliminating the elastic strands and allowing the 2 nonwoven facings to be bonded adhesively together, then slitting to the desired ruffle width.

The nonwoven used in this case was a 20 gsm (0.6 osy) spunbond/meltblown/spunbond laminate (SMS), although other nonwoven facings (i.e. 14 and 20 gsm (0.4 and 0.6 osy) spunbond) have shown similar results. In addition, the elastic strands decitex and spacing, the adhesive add-on and the percent stretch may also vary. The codes tested are as follows:
Code A: 10 cm (4.0") SMS/elastic strand laminate with no ruffle
Code B: 10 cm (4.0") SMS/elastic strand laminate with 0.6 cm (0.25") ruffle
Code C: 10 cm (4.0") SMS/elastic strand laminate with 1.3 cm (0.50") ruffle
Code D: 10 cm (4.0") SMS/elastic strand laminate with 1.9 cm (0.75") ruffle
Code E: 10 cm (4.0") SMS/elastic strand laminate with 2.5 cm (1.0") ruffle (desired design)
Code F: 13 cm (4.0") SMS/elastic strand laminate with no ruffle (this code was tested to eliminate the effect of sample width on the data).

Samples of each code are cut to at least 46 cm (18") in length (this provides for a testing length of 41 cm (16"), the approximate length needed to make a swimsuit top) and 2.5cm (an inch) in either side for attachment to the test template. The center of the width of each sample is determined as between the two outermost strands of elastics stands and a line is drawn down the entire center length of the sample. The ruffle width is not included in the measurement.

A piece of foam core or cork board is marked at 0, 41, 51 and 55 cm (0", 16", 20" and 21.5"). The 51 cm and 55 cm (20" and 21.5") marks represent the 41 cm (16") sample pulled to 25% and 35% respectively, which is the typical amount of stretch the material demonstrates when worn by a typical child.

Using a pin, one end of the material is attached into the board at the 0 cm (0") mark. Taking care to lay the material flat and straight, but without any elongation, the pin through the second end of the material is attached into the board at the **41** cm (16") mark. Once the material is attached, the end of the material at the **41** cm (16") mark is stretched to 51 cm (20") by removing the pin from the board and using the pin to pull the material to the 51 cm (20") mark. Any wrinkles are smoothed out around the pin and the sample is allowed to sit for 5 minutes.

After waiting for 5 minutes, the amount of curling of the lengthwise edges of the material is measured. This is accomplished with an inverted U-shaped clear template (approximately 5 cm (2.0) high by 15 cm (6.0") long) with a line drawn lengthwise at the centerline of the template. When placed over the sample, the centerline of the template should be directly over the centerline of the sample. In addition, the edge of the template (start of the centerline) should be placed at the exact center of the length of the sample (a line drawn of the board prior to testing to mark this point).

Measurement of amount of curl is accomplished by placing the U-shaped template over the sample so that the centerline of the template is directly above the centerline of the sample. Once the template is in place, measure the distance (in mm) from the centerline to each edge of the material should be measured and recorded. If the material has curled over enough to cover the centerline of the sample, the distance past the centerline should be added as well. In addition, it should be noted whether the material edge has just curled or has actually begun to fold over. After recording the measurements, the results for the ruffled material should be adjusted to take into account the width of the ruffle. This is accomplished by subtracting the width of the ruffle from the respective results of materials with ruffles.

After the measurements are completed at 25% stretch, the material pulled to the 55cm (21.5 inch) mark (35% elongation) using the pin again. The measurements of curl-over should be taken as described above and recorded. The test results are shown Table 1.

| Ruffle Width | | Percent | | Mean SAMPLE NUMBER | | | | | Distance (mm) |
|---|---|---|---|---|---|---|---|---|---|
| Sample (in) | | Side Stretch | | 1 | 2 | 3 | 4 | 5 | |
| 1 | 0.00 | A | 25 | 40.00 | 35.00 | 38.00 | 46.00 | 37.00 | 39.2 |
| 1 | 0.00 | Aa | 25 | 20.00 | 23.00 | 30.00 | 18.00 | 33.00 | 24.8 |
| | | | | | | | | | |
| 1 | 0.00 | A | 35 | 31.00 | 24.00 | 30.00 | 41.00 | 30.00 | 31.2 |
| 1 | 0.00 | Aa | 35 | 2.00 | 6.00 | 19.00 | 2.00 | 22.00 | 10.2 |
| | | | | | | | | | |
| 2 | 0.25 | A | 25 | 40.00 | 48.00 | 48.00 | 49.00 | 52.00 | 47.4 |
| 2 | 0.25 | B | 25 | 51.65 | 40.65 | 44.65 | 49.65 | 48.65 | 47.1 |
| 2 | 0.25 | A | 35 | 12.00 | 18.00 | 35.00 | 29.00 | 30.00 | 24.8 |
| 2 | 0.25 | B | 35 | 48.65 | 39.65 | 30.65 | 35.65 | 38.65 | 38.7 |
| | | | | | | | | | |
| 3 | 0.50 | A | 25 | 49.00 | 46.00 | 46.00 | 50.00 | 44.00 | 47.0 |
| 3 | 0.50 | B | 25 | 40.30 | 47.30 | 46.30 | 44.30 | 37.30 | 43.1 |
| 3 | 0.50 | A | 35 | 25.00 | 28.00 | 25.00 | 13.00 | 16.00 | 21.4 |
| 3 | 0.50 | B | 35 | 29.30 | 43.30 | 36.30 | 39.30 | 29.30 | 35.5 |
| | | | | | | | | | |
| 4 | 0.75 | A | 25 | 18.00 | 30.00 | 35.00 | 31.00 | 22.00 | 27.2 |
| 4 | 0.75 | B | 25 | 43.95 | 42.95 | 45.95 | 23.95 | 40.95 | 39.6 |
| 4 | 0.75 | A | 35 | -10.00 | 0.00 | 13.00 | 3.00 | 8.00 | 2.8 |
| 4 | 0.75 | B | 35 | 40.95 | 32.95 | 26.95 | 2.95 | 17.95 | 24.4 |
| | | | | | | | | | |
| 5 | 1.00 | A | 25 | 30.00 | 20.00 | 21.00 | 34.00 | 18.00 | 24.6 |
| 5 | 1.00 | B | 25 | 41.60 | 42.60 | 37,60 | 44.60 | 42.60 | 41.8 |
| 5 | 1.00 | A | 35 | 7.00 | -5.00 | -5.00 | 17.00 | 2.00 | 3.2 |
| 5 | 1.00 | B | 35 | 38.60 | 44.60 | 30.60 | 27.60 | 34.60 | 35.2 |
| | | | | | | | | | |
| 6 | 0.00 | A | 25 | 36.00 | 29.00 | 35.00 | 33.00 | 45.00 | 35.6 |
| 6 | 0.00 | Aa | 25 | 21.00 | 33.00 | 9.00 | 19.00 | 15.00 | 19.4 |
| 6 | 0.00 | A | 35 | 15.00 | 7.00 | 35.00 | 28.00 | 23.00 | 21.6 |
| 6 | 0.00 | Aa | 35 | 0.00 | 15.00 | -8.00 | -5.00 | 0.00 | 0.4 |

## Claims

1. A camisole garment (2) for wearing about the body comprising a body covering assembly (11) having an upper body opening (12) and a lower body opening (14) wherein each opening has an edge about its perimeter (4, 6), and two opposing end portions (48, 50) of the body covering assembly between the upper edge (4) and the lower edge (6) are engaged to form a body seam (42), the body covering assembly **characterised by**:
an elastic region (22) between the upper edge (4) and the lower edge (6);
a relatively inelastic lower edge region (30) between the elastic region and the lower edge wherein the lower edge region is relatively inelastic compared to the elastic region and the lower edge region further being from 0.64 to 10.2 cm (0.25 to 4.0 inches) in width;
a relatively inelastic upper edge region (24) between the elastic region and the upper edge region wherein the upper edge region is relatively inelastic compared to the elastic region, and the upper edge region further being from 0.64 to 10.2 cm (0.25 to 4.0 inches) in width;
at least one opening (32, 34) in the elastic region.

2. The camisole garment (2) of claim 1, further comprising a neckline edge fold (40) created by folding over the upper edge (4), the relatively inelastic upper edge region (24) and a portion of the elastic region (22) above the at least one opening (32, 34).

3. The camisole garment (2) of claim 1 or 2, wherein the body covering assembly (11) comprises:
at least two opposing openings (32, 34) in the elastic region (22).

4. The camisole garment (2) according to claim 1, 2 or 3 comprising an outer cover (16) and a bodyside liner (18), both of which cover a series of body elastics (20) which circumferentially surround the body to form the elastic region (22).

5. The camisole garment (2) according to any of claims 1 to 4, wherein the two opposing end portions (48, 50) are refastenably engaged to form a refastenable body seam (42).

6. The camisole garment (2) according to any of claims 1 to 4, wherein the two opposing end portions (48, 50) are non-refastenably engaged to form a non-refastenable body seam (42).

7. The camisole garment (2) according to any of claims 4 to 6, wherein the outer cover (16) is a gatherable material.

8. The camisole garment (2) according to any of claims 4 to 7 wherein the outer cover (16) is a woven material.

9. The camisole garment (2) according to any of claims 4 to 7, wherein the outer cover (16) is a nonwoven material.

10. The camisole garment (2) according to any of claims 4 to 7, wherein the outer cover (16) is a polymeric film material.

11. The camisole garment (2) according to any of claims 4 to 9, wherein the outer cover (16) is a fibrous material.

12. The camisole garment (2) according to any of claims 4 to 11, wherein the outer cover (16) is an elastic material.

13. The camisole garment (2) according to claim 11, wherein the outer cover (16) comprises acrylic polymer, polyester, polyamide, glass, polyethylene, polypropylene, rayon, cotton, silk, wool, pulp, paper, or a blend or combination of two or more of the foregoing.

14. The camisole garment (2) according to claim 10, wherein the outer cover (16) comprises acrylic polymer, polyester, polyamide, polyethylene, polypropylene, or a compatible mixture, blend or copolymer thereof.

15. The camisole garment (2) according to any of claims 4 to 7, wherein the outer cover (16) is a spunbonded polypropylene nonwoven material, meltblown polypropylene nonwoven material or spunbonded polypropylene nonwoven material laminate.

16. The camisole garment (2) according to claim 15, wherein the outer cover (16) has a basis weight of from 13 to 34 gsm (0.4 to 1.0 ounces per square yard), and contains 86% spunbonded polypropylene nonwoven material and 14% meltblown polypropylene nonwoven material.

17. The camisole garment (2) according to any of claims 4 to 16, wherein the bodyside liner (18) is a soft, flexible porous sheet which permits submersion in fresh water, salt water, chlorinated water or brominated water and thereafter retains its integrity.

18. The camisole garment (2) according to any of claims 4 to 17, wherein the bodyside liner (18) comprises a nonwoven or sheet of spunbonded, meltblown or bonded-carded web composed of polypropylene, polyethylene, polyester, rayon, or cotton filaments.

19. The camisole garment (2) of any of claims 4 to 18, wherein the body elastics (20) are elastic threads, yam rubber, flat rubber, elastic tape, polyurethane, or foamed elastic scrim.

20. The camisole garment (2) according to any of claims 4 to 19, wherein the body elastics (20) are elongated to between 50% to 300%.

21. The camisole garment (2) according to any preceding claim, wherein the body covering assembly (11) is made of materials having stretch characteristics such that the body covering assembly (11) is capable of between 50% to 300% elongation, and recovery, upon release of tension, of at least 80% of its elongation.

22. The camisole garment (2) according to any preceding claim, wherein the body covering assembly (11) is made of materials capable of stretching in one direction.

23. The camisole garment (2) according to any of claims 1 to 21, wherein the body covering assembly (11) is made of materials capable of stretching in two perpendicular directions.

24. A continuous process for the manufacture of a camisole garment (2) comprising:
a. providing at least a single layer web of fabric (3) including an upper edge (4), a lower edge (6), and a body covering assembly (11);
b. intermittently cutting the fabric (3), defining at least one opening (32,34) in the fabric (3) wherein each opening includes a top edge (36,38) adjacent to the upper edge (4) of the fabric (3);
c. folding at least a portion of the fabric (3) between at least one of the openings (32, 34) and the upper edge (4) of the fabric (3) back onto the body covering assembly (11) of the fabric (3) wherein at least one shoulder strap (26) is formed;
d. fastening the folded portion of the fabric (3) to the body covering assembly (11) of the fabric (3) to form a neckline fold (40);
e. cutting the fabric (3), defining discrete garment-sized pieces wherein each piece of fabric (3) includes at least one opening (32,34), at least one shoulder strap (26), and two opposing end portions (48,50);
f. folding the discrete garment-sized piece of fabric (3) whereby the two opposing end portions (48,50) are brought into contact with each other.

25. The continuous process according to claim 24, further comprising fastening the two opposing end portions (48,50) together to form a body seam (42).

26. The continuous process according to claim 24 or 25, wherein at least one pair of openings (32, 34) are cut into the fabric (3), and wherein each garment-sized piece of fabric (3) includes at least one pair of openings (32, 34) and at least one pair of shoulder straps (26,28).

27. The continuous process of claims 24 to 26 wherein the web of fabric (3) is a multi-layer laminate web of fabric.

28. The continuous process according to any of claims 24 to 27, further comprising tuming the folded discrete garment-sized piece of fabric (3) to move sideways.

29. The continuous process according to claims 24 to 28 further comprising cutting off excess fabric (3) remaining of the two opposing end portions (48,50) adjacent to the body seam (42).

30. The continuous process according to claims 24 to 29, wherein the body seam (42) is refastenable.

31. The continuous process according to claims 24 to 29, wherein the body seam (42) is non-refastenable.

## Patentansprüche

1. Hemdchen-Kleidungsstück (2) zum Tragen am Körper, das eine Körperumhüllungsanordnung (11) mit einer oberen Körperöffnung (12) und einer unteren Körperöffnung (14) umfasst, wobei jede Öffnung einen Rand um ihren Umfang (4, 6) herum aufweist und zwei einander gegenüberliegende Endabschnitte (48, 50) der Körperumhüllungsanordnung zwischen dem oberen Rand (4) und dem unteren Rand (6) in Eingriff sind, um eine Körpernaht (42) zu bilden, wobei die Körperumhüllungsanordnung **gekennzeichnet ist durch**:
einen elastischen Bereich (22) zwischen dem oberen Rand (4) und dem unteren Rand (6);
einen relativ unelastischen unteren Randbereich (30) zwischen dem elastischen Bereich und dem unteren Rand, wobei der untere Randbereich im Vergleich zu dem elastischen Bereich relativ unelastisch ist und der untere Randbereich des Weiteren zwischen 0,64 und 10,2 cm (0,25 und 4,0 lnch) breit ist;
einen relativ unelastischen oberen Randbereich (24) zwischen dem elastischen Bereich und dem oberen Randbereich, wobei der obere Randbereich im Vergleich zu dem elastischen Bereich relativ unelastisch ist und der obere Randbereich des Weiteren zwischen 0,64 und 10,2 cm (0,25 bis 4,0 Inch) breit ist;
wenigstens eine Öffnung (32, 34) in dem elastischen Bereich.

2. Hemdchen-Kleidungsstück (2) nach Anspruch 1, das des Weiteren eine Halslinienrand-Falte (40) umfasst, die geschaffen wird, indem der obere Rand (4), der relativ unelastische obere Randbereich (24) und ein Abschnitt des elastischen Bereiches (22) über der wenigstens einen Öffnung (32, 34) umgefaltet werden.

3. Hemdchen-Kleidungsstück nach Anspruch 1 oder 2, wobei die Körperumhüllungsanordnung (11) umfasst:
wenigstens zwei einander gegenüberliegende Öffnungen (32, 34) in dem elastischen Bereich (22).

4. Hemdchen-Kleidungsstück (2) nach Anspruch 1, 2 oder 3, die eine äußere Umhüllung (16) und eine Körperseiten-Auskleidung (18) umfasst, die beide eine Reihe von Körper-Elastiken (20) umhüllen, die den Körper in Umfangsrichtung umgeben, um den elastischen Bereich (22) zu bilden.

5. Hemdchen-Kleidungsstück (2) nach einem der Ansprüche 1 bis 4, wobei die zwei einander gegenüberliegenden Endabschnitte (48, 50) wieder verschließbar in Eingriff sind, um eine wieder verschließbare Körpernaht (42) zu bilden.

6. Hemdchen-Kleidungsstück (2) nach einem der Ansprüche 1 bis 4, wobei die zwei einander gegenüberliegenden Endabschnitte (48, 50) nicht wieder verschließbar in Eingriff sind, um eine nicht wieder verschließbare Körpernaht (42) zu bilden.

7. Hemdchen-Kleidungsstück (2) nach einem der Ansprüche 4 bis 6, wobei die äußere Umhüllung (16) ein zusammenziehbares Material ist.

8. Hemdchen-Kleidungsstück (2) nach einem der Ansprüche 4 bis 7, wobei die äußere Umhüllung (16) ein gewebtes Material ist.

9. Hemdchen-Kleidungsstück (2) nach einem der Ansprüche 4 bis 7, wobei die äußere Umhüllung (16) ein nicht gewebtes Material ist.

10. Hemdchen-Kleidungsstück (2) nach einem der Ansprüche 4 bis 7, wobei die äußere Umhüllung (16) ein Polymerfolienmaterial ist.

11. Hemdchen-Kleidungsstück (2) nach einem der Ansprüche 4 bis 9, wobei die äußere Umhüllung (16) ein Fasermaterial ist.

12. Hemdchen-Kleidungsstück (2) nach einem der Ansprüche 4 bis 11, wobei die äußere Umhüllung (16) ein elastisches Material ist.

13. Hemdchen-Kleidungsstück (2) nach Anspruch 11, wobei die äußere Umhüllung (16) Acrylpolymer, Polyester, Polyamid, Glas, Polyethylen, Polypropylen, Reyon, Baumwolle, Seide, Wolle, Zellstoff, Papier oder ein Gemisch bzw. eine Kombination aus zwei oder mehr der genannten Bestandteile umfasst.

14. Hemdchen-Kleidungsstück (2) nach Anspruch 10, wobei die äußere Umhüllung (16) Acrylpolymer, Polyester, Polyamid, Polyethylen, Polypropylen oder ein kompatibles Gemisch, eine Mischung oder ein Copolymer davon umfasst.

15. Hemdchen-Kleidungsstück (2) nach einem der Ansprüche 4 bis 7, wobei die äußere Umhüllung (16) ein spunbonded Polypropylen-Vliesmaterial, Meltblown- Polypropylen-Vliesmaterial oder spunbonded Polypropylen-Vliesmaterial-Laminat ist.

16. Hemdchen-Kleidungsstück (2) nach Anspruch 15, wobei die äußere Umhüllung (16) eine Flächenmasse zwischen 13 und 34 glm² (0,4 bis 1,0 ounces per square yard) hat und 86% spunbonded Polypropylen-Vliesmaterial sowie 14% Meltblown- Polypropylen-Vliesmaterial enthält.

17. Hemdchen-Kleidungsstück (2) nach einem der Ansprüche 4 bis 16, wobei die Körperseiten-Auskleidung (18) eine weiche, flexible, poröse Lage ist, die Eintauchen in Süßwasser, Salzwasser, chloriertes Wasser und bromiertes Wasser ermöglicht und danach unversehrt bleibt.

18. Hemdchen-Kleidungsstück (2) nach einem der Ansprüche 4 bis 17, wobei die Körperseiten-Auskleidung (18) ein Vlies oder eine Lage einer spunbonded, Meltblownoder gebonded-kardierten Bahn umfasst, die aus Polypropylen-, Polyethylen-, Polyester-, Reyon- oder Baumwollfäden besteht.

19. Hemdchen-Kleidungsstück (2) nach einem der Ansprüche 4 bis 18, wobei die Körper-Elastiken (20) elastische Fäden, Garngummi, Flachgummi, elastisches Band, Polyurethan oder verschäumter elastischer Gitterstoff sind.

20. Hemdchen-Kleidungsstück (2) nach einem der Ansprüche 4 bis 19, wobei die Körper-Elastiken (20) auf zwischen 50% und 300% gedehnt sind.

21. Hemdchen-Kleidungsstück nach einem der vorangehenden Ansprüche, wobei die Körperumhüllungsanordnung (11) aus Materialien besteht, die Streckeigenschaften haben, so dass sich die Körperumhüllungsanordnung (11) auf zwischen 50% und 300% dehnen und beim Ablassen der Spannung auf wenigstens 80% ihrer Dehnung rückverformen kann.

22. Hemdchen-Kleidungsstück (2) nach einem der vorangehenden Ansprüche, wobei die Körperumhüllungsanordnung (11) aus Materialien besteht, die in einer Richtung gestreckt werden können.

23. Hemdchen-Kleidungsstück (2) nach einem der Ansprüche 1 bis 21, wobei die Körperumhüllungsanordnung (11) aus Materialien besteht, die in zwei senkrechten Richtungen gestreckt werden können.

24. Kontinuierliches Verfahren zur Herstellung eines Hemdchen-Kleidungsstücks (2), das umfasst:
a) Bereitstellen wenigstens einer einschichtigen Bahn aus Gewebe (3), die einen oberen Rand (4), einen unteren Rand (6) und eine Körperumhüllungsanordnung (11) enthält;
b) intermittierendes Schneiden des Gewebes (3), so dass wenigstens eine Öffnung (32, 34) in dem Gewebe (3) ausgebildet wird, wobei jede Öffnung einen obersten Rand (36, 38) an den oberen Rand (4) des Gewebes (3) angrenzend enthält;
c) Umfalten wenigstens eines Abschnitts des Gewebes (3) zwischen wenigstens einer der Öffnungen (32, 34) und dem oberen Rand (4) des Gewebes (3) auf die Körperumhüllungsanordnung (11) des Gewebes (3), wobei wenigstens ein Schulterträger (26) ausgebildet wird;
d) Befestigen des umgefalteten Abschnitts des Gewebes (3) an der Körperumhüllungsanordnung (11) des Gewebes (3), um eine Halslinienfalte (40) auszubilden;
e) Schneiden des Gewebes, so dass einzelne Teile in Kleidungsstückgröße ausgebildet werden, wobei jedes Teil des Gewebes (3) wenigstens eine Öffnung (32, 34), wenigstens einen Schulterträger (26) und zwei einander gegenüberliegende Endabschnitte (48, 50) enthält;
f) Umfalten des einzelnen Teils des Gewebes (3) in Kleidungsstückgröße, so dass die zwei einander gegenüberliegenden Endabschnitte (48, 50) miteinander in Kontakt gebracht werden.

25. Kontinuierliches Verfahren nach Anspruch 24, das des Weiteren das Befestigen der zwei einander gegenüberliegenden Endabschnitte (48, 50) aneinander umfasst, um eine Körpernaht (42) zu bilden.

26. Kontinuierliches Verfahren nach Anspruch 24 oder 25, wobei wenigstens ein Paar Öffnungen (32, 34) in das Gewebe (3) geschnitten wird und wobei jedes Teil des Gewebes (3) in Kleidungsstückgröße wenigstens ein Paar Öffnungen (32, 34) und wenigstens ein Paar Schulterträger (26, 28) enthält.

27. Kontinuierliches Verfahren nach den Ansprüchen 24 bis 26, wobei die Bahn aus Gewebe (3) eine mehrschichtige Laminatbahn aus Gewebe ist.

28. Kontinuierliches Verfahren nach einem der Ansprüche 24 bis 27, das des Weiteren das Umdrehen des gefalteten einzelnen Teils aus Gewebe (3) in Kleidungsstückgröße zur seitlichen Bewegung umfasst.

29. Kontinuierliches Verfahren nach den Ansprüchen 24 bis 28, das des Weiteren das Abschneiden von überschüssigem Gewebe (3) umfasst, das an den zwei einander gegenüberliegenden Endabschnitten (48, 50) an die Körpernaht (42) angrenzend verbleibt.

30. Kontinuierliches Verfahren nach den Ansprüchen 24 bis 29, wobei die Körpernaht (42) wieder verschließbar ist.

31. Kontinuierliches Verfahren nach den Ansprüchen 24 bis 29, wobei die Körpernaht (42) nicht wieder verschließbar ist.

## Revendications

1. Camisole (2) à porter sur le corps, comprenant un assemblage couvrant le corps (11) ayant une ouverture corporelle supérieure (12) et une ouverture corporelle inférieure (14), chaque ouverture ayant un bord le long de son périmètre (4,6), et deux portions d'extrémité opposées (48,50) de l'assemblage couvrant le corps entre le bord supérieur (4) et le bord inférieur (6) sont en prise pour former une couture corporelle (42), l'assemblage couvrant le corps étant **caractérisé par** :
une région élastique (22) entre le bord supérieur (4) et le bord inférieur (6) ;
une région de bord inférieur (30) relativement inélastique, entre la région élastique et le bord inférieur, ladite région de bord inférieur étant relativement inélastique par comparaison avec la région élastique, et la région de bord inférieur ayant en outre une largeur comprise entre 0,64 à 10,2 cm (entre 0,25 et 4,0 pouces) ;
une région de bord supérieur (24) relativement inélastique, entre la région élastique et le bord supérieur, ladite région de bord supérieur étant relativement inélastique par comparaison avec la région élastique, et la région de bord supérieur ayant en outre une largeur comprise entre 0,64 et 10,2 cm (entre 0,25 et 4,0 pouces) ;
au moins une ouverture (32,34) dans la région élastique.

2. Camisole (2) selon la revendication 1, comprenant en outre un pli de bord d'encolure (40) créé en repliant le bord supérieur (4), la région de bord supérieur (24) relativement élastique et une portion de la région élastique (22) au-dessus de ladite au moins une ouverture (32,34).

3. Camisole (2) selon la revendication 1 ou 2, dans laquelle l'assemblage couvrant le corps (11) comprend :
au moins deux ouvertures (32,34) opposés dans la région élastique (22).

4. Camisole (2) selon la revendication 1, 2 ou 3, comprenant une feuille de couverture extérieure (16) et une doublure côté corporel (18), qui toutes deux couvrent une série d'élastiques corporels (20) entourant circonférentiellement le corps pour former la région élastique (22).

5. Camisole (2) selon l'une quelconque des revendications 1 à 4, dans laquelle les deux portions d'extrémité opposées (48,50) viennent en prise réattachable pour former une couture corporelle (42) réattachable.

6. Camisole (2) selon l'une quelconque des revendications 1 à 4, dans laquelle les deux portions d'extrémité opposées (48,50) viennent en prise non-réattachable pour former une couture corporelle (42) non-réattachable.

7. Camisole (2) selon l'une quelconque des revendications 4 à 6, dans laquelle la feuille de couverture extérieure (16) est un matériau fronçable.

8. Camisole (2) selon l'une quelconque des revendications 4 à 7, dans laquelle la feuille de couverture extérieure (16) est un matériau tissé.

9. Camisole (2) selon l'une quelconque des revendications 4 à 7, dans laquelle la feuille de couverture extérieure (16) est un matériau non-tissé.

10. Camisole (2) selon l'une quelconque des revendications 4 à 7, dans laquelle la feuille de couverture extérieure (16) est un matériau en film polymère.

11. Camisole (2) selon l'une quelconque des revendications 4 à 9, dans laquelle la feuille de couverture extérieure (16) est un matériau fibreux.

12. Camisole (2) selon l'une quelconque des revendications 4 à 11, dans laquelle la feuille de couverture extérieure (16) est un matériau élastique.

13. Camisole (2) selon la revendication 11, dans laquelle la feuille de couverture extérieure (16) comprend un polymère acrylique, un polyester, un polyamide, du verre, un polyéthylène, un polypropylène, de la rayonne, du coton, de la soie, de la laine, de la pâte, du papier ou un mélange ou une combinaison de deux, ou davantage, des matériaux précités.

14. Camisole (2) selon la revendication 10, dans laquelle la feuille de couverture extérieure (16) comprend un polymère acrylique, un polyester, un polyamide, un polyéthylène, un polypropylène, ou un mélange ou une alliance compatible ou copolymère de ces matériaux.

15. Camisole (2) selon l'une quelconque des revendications 4 à 7, dans laquelle la feuille de couverture extérieure (16) est un matériau non-tissé de polypropylène obtenu par filage-nappage, un matériau non-tissé de polypropylène obtenu par extrusion-soufflage ou un stratifié de matériau non-tissé de polypropylène obtenu par filage-nappage.

16. Camisole (2) selon la revendication 15, dans laquelle la feuille de couverture extérieure (16) a une masse surfacique comprise entre 13 et 34 g/m² (0,4 à 1,0 once/yard²), et contient 86 % d'un matériau non-tissé en polypropylène obtenu par filage-nappage et 14 % d'un matériau non-tissé en polypropylène obtenu par extrusion-soufflage.

17. Camisole (2) selon l'une quelconque des revendications 4 à 16, dans laquelle la doublure côté corporel (18) est une feuille poreuse, souple et douce qui supporte une immersion dans de l'eau douce, de l'eau salée, de l'eau chlorée ou de l'eau bromée, tout en conservant ensuite son intégrité.

18. Camisole (2) selon l'une quelconque des revendications 4 à 17, dans laquelle la doublure côté corporel (18) comprend un matériau non-tissé ou une feuille d'un voile obtenu par filage-nappage, extrusion-soufflage, ou cardé-lié composé de filaments de polypropylène, polyéthylène, polyester, rayonne ou coton.

19. Camisole (2) selon l'une quelconque des revendications 4 à 18, dans laquelle les élastiques corporels (20) sont des fils élastiques, du caoutchouc en fil, du caoutchouc plat, du ruban élastique, du polyuréthane ou une grille élastique alvéolée.

20. Camisole (2) selon l'une quelconque des revendications 4 à 19, dans laquelle les élastiques corporels (20) sont allongés jusqu'à une valeur comprise entre 50 % et 300 %.

21. Camisole (2) selon l'une quelconque des revendications précédentes, dans laquelle l'assemblage couvrant le corps (11) est fait de matériaux ayant des caractéristiques d'extensibilité telles que l'assemblage couvrant le corps (11) est capable d'un allongement compris entre 50 % et 300 %, et d'avoir une récupération, lorsque cesse la tension, d'au moins 80 % de son allongement.

22. Camisole (2) selon l'une quelconque des revendications précédentes, dans laquelle l'assemblage couvrant le corps (11) est fait de matériaux capables de s'étirer dans une direction.

23. Camisole (2) selon l'une quelconque des revendications 1 à 21, dans laquelle l'assemblage couvrant le corps (11) est fait de matériaux capables de s'étirer dans deux directions perpendiculaires.

24. Procédé continu pour la fabrication d'une camisole (2) comprenant :
a. la fourniture d'au moins un voile à couche unique d'étoffe (3) comprenant un bord supérieur (4), un bord inférieur (6) et un assemblage couvrant le corps (11) ;
b. la découpe intermittente de l'étoffe (3), définissant au moins une ouverture (32,34) dans l'étoffe (3), chaque ouverture comprenant un bord supérieur (36,38) adjacent au bord supérieur (4) de l'étoffe (3) ;
c. le repliage d'au moins une portion de l'étoffe (3) entre l'une au moins des ouvertures (32,34) et le bord supérieur (4) de l'étoffe (3) sur l'assemblage couvrant le corps (11) de l'étoffe (3), grâce à quoi au moins une bride d'épaule (26) est formée ;
d. la fixation de la portion repliée de l'étoffe (3) à l'assemblage couvrant le corps (11) de l'étoffe (3) pour former un pli d'encolure (40) ;
e. la découpe de l'étoffe (3) pour définir des morceaux séparés de la taille d'un vêtement, chaque morceau d'étoffe (3) comprenant au moins une ouverture (32,34), au moins une bride d'épaule (26) et deux portions d'extrémité opposées (48,50) ;
f. le pliage du morceau séparé d'étoffe (3) de la taille d'un vêtement, grâce à quoi les deux portions d'extrémité opposées (48,50) sont amenées au contact l'une de l'autre.

25. Procédé continu selon la revendication 24, comprenant en outre la fixation des deux portions d'extrémité opposées (48,50) l'une à l'autre pour former une couture corporelle (42).

26. Procédé continu selon la revendication 24 ou 25, dans lequel l'une au moins des paires d'ouvertures (32,34) est découpée dans l'étoffe (3), et dans lequel chaque morceau d'étoffe (3) de la taille d'un vêtement comprend au moins une paire d'ouvertures (32,34) et au moins une paire de brides d'épaule (26,28).

27. Procédé continu selon les revendications 24 à 26, dans lequel le voile d'étoffe (3) est un voile d'étoffe stratifiée à couches multiples.

28. Procédé continu selon Tune quelconque des revendications 24 à 27, comprenant en outre le fait de tourner le morceau séparé et plié d'étoffe (3) de la taille d'un vêtement pour le déplacer latéralement.

29. Procédé continu selon les revendications 24 à 28, comprenant en outre la découpe de l'excès d'étoffe (3) restant des deux portions d'extrémité opposées (48,50) adjacentes à la couture corporelle (42).

30. Procédé continu selon les revendications 24 à 29, dans lequel la couture corporelle (42) est réattachable.

31. Procédé continu selon les revendications 24 à 29, dans lequel la couture corporelle (42) est non-réattachable.
